

# UNITED STATES PATENT OFFICE.

MAX MÜLLER, OF FINKENWALDE, NEAR STETTIN, GERMANY.

## PROCESS FOR THE MANUFACTURE OF ARTIFICIAL THREADS, RIBBONS, FILMS, OR PLATES, FROM VISCOSE.

1,386,521.

Specification of Letters Patent.

Patented Aug. 2, 1921.

No Drawing.

Application filed July 17, 1920. Serial No. 397,144.

*To all whom it may concern:*

Be it known that I, MAX MÜLLER, a citizen of the Free State of Prussia, in the German Republic, residing at Finkenwalde, near 5 Stettin, in the Free State of Prussia, Germany, have invented Improvements in and Relating to a Process for the Manufacture of Artificial Threads, Ribbons, Films, or Plates from Viscose, for which application 10 was filed in Germany Sept. 6, 1918; and I do hereby declare the following to be a full, clear, and exact description of the same.

Viscose solutions have often been used for the manufacture of threads, films and the 15 like. In most cases precipitating baths have been employed containing dissolved sulfuric acid and a salt. Glucose additions and glycerin with or without an addition of sulfates of ammonium, magnesium and the like have 20 also been used.

In the manufacture of these artificial substances, which must show an especially high degree of brilliancy in order to be useful from an economic point of view, the recovery 25 of hydro cellulose structures was essential.

It has now been found that especially valuable products may be obtained in the manufacture of the so-called staple-fiber and 30 other viscose structures if the waste lye of the sulfite cellulose production is used in the precipitating bath.

The presence of hexosene and pentosene or of tanning and non-tanning substances in 35 this sulfite lye and the behavior of the waste lye with regard to mineral acids and salts have evidently contributed to this surprising result. The dark color of the waste sulfite lye does not affect the process but a "clearing-up" sufficient for spinning purposes may 40 be obtained.

It has also been found that the waste sulfite lye may with equal advantage be used as first element of the acid bath if other 45 viscose products not produced by spinning are to be precipitated and fixed from the viscose solutions.

In the manufacture of artificial threads and staple-fibers preferably a waste lye is 50 used which by suitable means such as sulfuric acid, oxalic acid or sodium carbonate has been freed of lime and is condensed by evaporation. This waste lye is varied to a favorable acid content with sulfurous acid, 55 sulfuric acid or hydrochloric-acid, the

amount of acid being regulated during spinning.

For example a spinning bath is used which is made by mixing together 30 parts of extract of sulfite of 30° Be. 11 parts of 60 sulfuric acid of 66% and 59 parts of water. Precipitated sulfate of lime is of course removed.

The use of the waste lye of sodium sulfite which has been produced either directly by 65 boiling of wood with the lye of sodium bisulfite or by converting of sodium salts from the waste lye of lime, has proven especially advantageous.

The waste lye obtained by the manufacture 70 of sulfite spirits is also very useful, in which case however a greater amount of the sulfite washes are to be employed. (For the example given above, 35 to 40 parts are necessary.)

Lastly, it has been found that an addition 75 of a hardening agent to the precipitating bath of the waste lye of sulfite has an advantageous effect upon the quality of the product. In order to obtain special effects 80 hardening agents, such as formaldehyde sulfate of alumina and the like, may be used and different additions to the precipitating bath, such as animal glue, sea-weed mucilages and so forth, may be made.

The water sensibility and the coloring 85 ability of the cellulose structures may in this way be especially favorably effected.

As has been mentioned above mineral acids and also acid salts are well known as 90 precipitating bath for viscose. In practice, heretofore, the "Muller-bath" has been used mainly. In the industry this precipitating bath was made by dissolving in water the bisulfate obtained as a waste product and adding sulfuric acid until the required amount of sulfuric acid is present in the bath.

According to this invention it is now possible to replace the bisulfate which is difficult to obtain as a waste product at the present by waste sulfite lye which is substantially valueless. It was not to be expected that such a complicated waste lye with its dark color (nearly black) and with 100 all its impurities could be used for the manufacture of artificial silk. It was, instead, a new and unexpected result.

The action resulting from the substance dissolved in the waste sulfite lye is not yet 110

quite explained. The glycose substances (hexosene and pentosene) protect the thread or film produced against a too energetical action of the sulfuric acid while the acid sulfites of the lye slowly decompose, giving up sulfurous acid which besides the added mineral acid (sulfuric acid) effects precipitating and fixing of the fiber.

According to this invention, the bisulfite, 10 which is now difficult to obtain, and the neutral sulfate contained therein is replaced by the waste lye of sulfite; and further, a portion of the free sulfuric acid of the bisulfite is replaced by sulfurous acid.

15 I claim as my invention:

1. The herein-described process of manufacturing artificial threads and other structures from viscose which consists in squirting the viscose into a precipitating bath 20 comprising acidified waste lye of sulfite cellulose.

2. The herein-described process of manufacturing artificial threads and other structures from viscose which consists in squirting 25 the viscose into a precipitating bath comprising waste lye of sulfite cellulose to which an acid salt has been added.

3. The herein-described process of manufacturing artificial threads and other structures 30 from viscose which consists in squirting the viscose into a precipitating bath comprising waste lye of sulfite cellulose to which a mineral acid has been added.

4. The herein-described process of manufacturing artificial threads and other structures 35 from viscose which consists in squirting the viscose into a precipitating bath comprising waste lye of sulfite cellulose to which sulfuric acid has been added.

40 5. The herein-described process of manufacturing artificial threads and other structures from viscose which consists in squirting the viscose into a precipitating bath com-

prising acidified waste lye of sodium sulfite.

6. The herein-described process of manufacturing artificial threads and other structures from viscose which consists in squirting the viscose into a precipitating bath comprising the waste lye obtained by the 50 manufacture of sulfite spirits.

7. The herein-described process of manufacturing artificial threads and other structures from viscose which consists in squirting the viscose into a precipitating bath 55 comprising waste lye of sulfite cellulose to which an acid and hardening agents have been added.

8. The herein-described process of manufacturing artificial threads and other structures from viscose which consists in squirting the viscose into a precipitating bath comprising waste lye of sulfite cellulose to which an acid and formaldehyde have been added.

9. The herein-described process of manufacturing artificial threads and other structures from viscose which consists in squirting the viscose into a precipitating bath comprising waste lye of sulfite cellulose to which an acid and hardening agents and 70 other additions to obtain special effects have been added.

10. The herein-described process of manufacturing artificial threads and other structures from viscose which consists in squirting 75 the viscose into a precipitating bath comprising waste lye of sulfite cellulose to which an acid and hardening agents and glue have been added.

In testimony whereof I have signed my 80 name to this specification in the presence of two subscribing witnesses.

Dr. MAX MÜLLER.

Witnesses:

RUDOLF BAUMGARD,  
RICHARD KÜKEN.